

Jan. 14, 1964

C. D. COXE

3,117,894

HARDENING SPRING BY INTERNAL OXIDATION

Filed Oct. 8, 1959

Fig. 1



Fig. 2



Fig. 3

Fig. 4



INVENTOR.  
Charles D. Coxe

BY

Pollard Johnston Smyth Polkerton  
ATTORNEYS

## 1

3,117,894

HARDENING SPRING BY INTERNAL  
OXIDATION

Charles D. Coxe, Fairfield, Conn., assignor to Handy and Harman, Fairfield, Conn., a corporation of New York  
Filed Oct. 8, 1959, Ser. No. 845,227  
3 Claims. (Cl. 148—11.5)

This invention relates to springs and particularly those requiring high electrical or thermal conductivities.

In spring members which are normally under load, such as electrical relay springs, vacuum tube clips, spring collet fingers and the like, it is desirable to have a spring material with high electrical or thermal conductivity, as the service may require. Such a spring must be able to withstand high temperatures and yet retain its resilience and high elastic limit.

It is known that metals such as silver or copper can be alloyed with small amounts of metals having a high heat of oxide formation, such as magnesium, beryllium, or aluminum, and then can be hardened by heating the alloy in an oxidizing environment to form internally oxidized alloys having high strength, conductivity, and extraordinary ability to retain a substantial measure of these physical properties at elevated temperature. Their room temperature properties are unaffected by heating to temperatures that would completely anneal or soften conventional metallic alloys not internally oxidizable. Such internally oxidized alloys are comprised of substantially pure metallic matrices having dispersed therein very fine (submicron size) oxide particles.

While the tensile properties of such internally oxidized alloys are such as would make their use in spring members desirable, it has been found that such springs are subject to spontaneous cracking under constant load, with practically no elongation.

One of the objects of the invention is to provide a process for making spring members which will not spontaneously crack or fail when under constant load and will not lose their resilience after heating to temperatures that would completely anneal conventional spring materials.

Another of the objects of the invention is to provide a spring member which can be used under a continuous load without failure.

In one aspect of the invention, a polycrystalline metal alloy capable of being internally oxidized is subjected to an oxidizing environment. The internally oxidized polycrystalline alloy is plastically deformed 50% or more, and then formed into a spring. After plastic deformation, the alloy preferably is subjected to an annealing operation. If the plastic deformation is at least 75%, it is not always necessary to anneal.

These and other objects, advantages and features of the invention will become apparent from the following description and drawings.

In the drawings:

FIG. 1 shows an enlarged view of a strip of metal and schematically shows plastic deformation thereof;

## 2

FIG. 2 shows a test strip of metal bowed into a spring; FIG. 3 is similar to FIG. 2 except the spring is shown broken;

5 FIG. 4 shows one use of a spring member made in accordance with the invention, such merely being an example.

The invention involves springs made of solid solution alloys which consist of relatively non-oxidizable solvent metal alloy capable of diffusing oxygen and solute metal 10 which forms stable oxides. Internal oxidation is accomplished by subjecting such a solid solution alloy or internally oxidizable alloy or material to an environment of an oxygen containing gas or media at elevated temperatures. Such an environment is one that is oxidizing to the solute metals but non-oxidizing to the solvent metals. The hardening of the alloy is the result of internal oxidation wherein very small refractory oxide particles are precipitated in the matrix.

20 As an example, a leaf spring of the alloy Ag 99.5% Mg 0.3% Ni 0.2% may be prepared and rolled to a strip 0.012" thick as shown in edge view in FIGURE 1. This spring strip may then be hardened by heating in air at 1350° F. for about 45 minutes. If this spring is then sprung into a bow and restrained at the ends so that the outer fibers of the spring are under tension, the spring will frequently fracture, as in FIGURE 3, on standing at room temperature, and will fracture in almost every case when subjected to temperatures in the range of 500° to 1000° F. while under load. Attempts to alleviate cracking of the spring by reducing the oxide content undesirably lowers the tensile properties and this is not satisfactory for a spring normally under load.

35 As one example of the invention, a leaf spring was made of an alloy composed of Ag 99.5% Mg 0.3% Ni 0.2% rolled to a strip 0.048" in thickness and then hardened by heating in air at 1350° F. for about 9 hours, the thicker material requiring a longer time for oxygen penetration. It was then cold rolled to 0.012" and tested by being sprung into a bow, as seen in FIG. 2. It was found to no longer be crack sensitive and to withstand heating to 1000° F. under load without failure. An illustration of 40 a failed spring is seen in FIG. 3. The invention has been found to be particularly efficacious when the oxidizable metal content is over 0.2%. Annealing can be carried out at a temperature in the range of 1000° F. to 1400° F.

45 The effect of cold working various amounts subsequent to oxidation is shown in the following table which tabulates the tensile properties and cracking performance of spring strips that have been cold worked various amounts after hardening. In these tests, the bowed leaf springs were held 20 hours at room temperature. Those surviving this test were then placed in an oven at 500° F. for 6 hours, where additional failures occurred. The survivors were then heated to 1000° F. for 6 hours, where additional failures occurred. Those failing at room temperature were termed poor, those failing at 500° F. fair, those failing at 1000° F. good, and those surviving the 1000° F. 50

test excellent. The test results under this procedure, together with strengths obtained, were as follows:

tential pressure that will selectively oxidize Be without causing the copper to scale excessively.

Table I

| Treatment No. | Treatment                                                                | Testing Direction, Longitudinal or Transverse | Yield Strength $\times 1,000$ p.s.i. | Tensile Strength $\times 1,000$ p.s.i. | Elong., percent | Cracking Test |
|---------------|--------------------------------------------------------------------------|-----------------------------------------------|--------------------------------------|----------------------------------------|-----------------|---------------|
| I             | Cold Rolled .600" to .012"; Oxidized 1,350° F.                           | (L)                                           | 75.0                                 | 79.0                                   | 7               | Poor.         |
| II            | Cold Rolled .600" to .016"; Oxidized 1,350° F.; Cold Rolled .012" (25%). | (L)                                           | 64.6                                 | 66.5                                   | 6               | Good.         |
| III           | II plus anneal 1,350° F.                                                 | (T)                                           | 78.5                                 | 84.1                                   | 2               | Poor.         |
| IV            | Cold Rolled .600" to .024"; Oxidized 1,350° F.; Cold Rolled .012" (50%). | (L)                                           | 69.1                                 | 72.8                                   | 3               | Do.           |
| V             | IV plus anneal 1,350° F.                                                 | (T)                                           | 77.6                                 | 78.7                                   | 3               | Fair.         |
| VI            | Cold Rolled .600" to .048"; Oxidized 1,350° F.; Cold Rolled .012" (75%). | (L)                                           | 73.1                                 | 75.7                                   | 2               | Do.           |
| VII           | VI plus anneal 1,375° F.                                                 | (T)                                           | 77.1                                 | 82.8                                   | 1               | Excellent.    |
|               |                                                                          | (T)                                           | 69.3                                 | 73.0                                   | 14              | Fair.         |
|               |                                                                          | (L)                                           | 75.0                                 | 77.8                                   | 8               | Excellent.    |
|               |                                                                          | (T)                                           | 77.5                                 | 79.1                                   | 2.5             | Do.           |
|               |                                                                          | (L)                                           | 67.1                                 | 76.7                                   | 3               | Do.           |
|               |                                                                          | (T)                                           | 67.0                                 | 76.1                                   | 8               | Do.           |
|               |                                                                          | (L)                                           | 68.9                                 | 72.2                                   | 8               | Do.           |
|               |                                                                          | (T)                                           | 69.5                                 | 77.2                                   | 11              | Do.           |

These tests were repeated on material which, during the initial cold rolling before oxidation, was annealed in process before the last 50% reduction prior to oxidation to reduce the directionality of the strength properties, i.e., to produce less preferred orientation of crystallographic axis in the direction of rolling.

The tendency for delayed brittle fracture in stress, as oxidized (not cold worked) alloy springs increases as the oxidizable element increases, or as the strength increases. Generally, when the as oxidized strength is well below 60,000 p.s.i., delayed brittle fracture does not occur, and when it is well above 60,000 p.s.i., it will nearly always

Table II

| Treatment No. | Treatment                  | Testing Direction, Longitudinal or Transverse | Yield Strength $\times 1,000$ p.s.i. | Tensile Strength $\times 1,000$ p.s.i. | Elong., percent | Cracking Test |
|---------------|----------------------------|-----------------------------------------------|--------------------------------------|----------------------------------------|-----------------|---------------|
| I-A           | (as oxidized)              | (L)                                           | 70.0                                 | 73.1                                   | 6               | Good.         |
|               |                            | (T)                                           | 68.5                                 | 70.0                                   | 11              | Fair.         |
| II-A          | 25% C.R. after oxidizing   | (L)                                           | 75.9                                 | 80.5                                   | 2               | Do.           |
|               |                            | (T)                                           | 74.9                                 | 80.8                                   | 3               | Poor.         |
| III-A         | II-A plus 1,350° anneal    | (L)                                           | 74.5                                 | 76.8                                   | 12              | Fair.         |
|               |                            | (T)                                           | 77.0                                 | 77.2                                   | 8               | Do.           |
| IV-A          | 50% C.R. after oxidizing   | (L)                                           | 75.0                                 | 77.5                                   | 1               | Excellent.    |
|               |                            | (T)                                           | 73.4                                 | 74.3                                   | 4               | Poor.         |
| V-A           | IV-A plus anneal 1,350° F. | (L)                                           | 78.5                                 | 79.7                                   | 7               | Excellent.    |
|               |                            | (T)                                           | 69.3                                 | 72.0                                   | 5               | Do.           |
| VI-A          | 75% C.R. after oxidizing   | (L)                                           | 72.5                                 | 74.6                                   | 10              | Do.           |
|               |                            | (T)                                           | 77.9                                 | 80.4                                   | 7               | Do.           |
| VII-A         | VI-A plus 1,350° Anneal    | (L)                                           |                                      |                                        |                 |               |
|               |                            | (T)                                           |                                      |                                        |                 |               |

It will be noted that 25% cold rolling after oxidizing reduced resistance to cracking, 50% reduction improved it in some cases, and 50% reduction plus annealing eliminated it as did 75% reduction and 75% reduction plus annealing.

Heretofore, the cracking of internally oxidized polycrystalline metal has seriously hindered its use as springs. This improvement makes possible much more extensive use of springs of such material at elevated temperatures and at higher loads.

The process of severe plastic deformation thus overcomes a basic defect in internally oxidized polycrystalline alloys, but it is important that the plastic deformation be substantial—a little, 25%, under the above experimental conditions was worse than none. The limits may differ for other alloys and processing details.

Annealing appears to be necessary to avoid brittleness in 50% cold worked material, but not in 75% cold worked material. However, if a spring member is to be further shaped or formed after cold rolling, the added ductility obtained by annealing will facilitate operations such as bending to the desired form of leaf springs, or the winding of coil springs. Flat, cantilever type springs, cold worked 75%, need not be annealed.

Similar results were obtained with an alloy of copper with 0.1% to 0.2% of beryllium, oxidized at 1600° F. in a pack of  $\text{Cu}_2\text{O}$  which serves to furnish oxygen at a par-

50 occur. Hence the invention is particularly useful for springs stronger than 60,000 p.s.i., and especially in springs having 70,000 p.s.i. tensile strength. The lower limit of magnesium in silver for which the invention is effective under any condition is about 0.1%. Similarly, it appears that about 0.05% Be in copper is a minimum alloy that will benefit from the invention. When Be in copper exceeds about 0.25% and Mg in silver exceeds about 0.35%, the oxidized alloy becomes too brittle to cold work satisfactorily. Thus, in an Ag alloy, the Mg should be between about 0.1% and 0.35%. In a Cu alloy of the type described, the Be should be between about 0.05% and 0.25%.

55 Other matrix metals capable of having their solute metal internally oxidized may be used, such as for example palladium and nickel.

FIG. 4 shows one type of spring employing the present invention wherein the spring clip members 10 and 11 are arranged to grip an electronic tube 12. The clip can be formed from the rolled strip material. The spring can be brazed (1200°–1400° F.) to a dissipating base member 13 (heat sink), without affecting the properties of the spring.

60 It should be apparent that details of the invention can be varied without departing from the spirit of the invention except as defined in the appended claims.

What is claimed is:

1. The process of making a spring of polycrystalline metal alloy hardenable by internal oxidation, said alloy having a solvent metal selected from the group consisting of silver, copper, palladium and nickel and an oxidizable metal dissolved therein in an amount ranging between 0.05% and 0.35%, comprising the steps of subjecting said alloy at elevated temperature in the range below the melting point of said solvent metal and above the minimum temperature for effective oxidation of said oxidizable metal to an oxygen containing environment to oxidation harden said alloy, decreasing the cross-sectional area of the oxidation hardened metal by cold working at least 50%, annealing the cold worked oxidation hardened metal, and forming a spring therefrom.

2. The process of making a spring of polycrystalline metal alloy hardenable by internal oxidation, said alloy having a solvent metal selected from the group consisting of silver, copper, palladium and nickel and an oxidizable metal dissolved therein in an amount ranging between 0.05% and 0.35%, comprising the steps of subjecting said alloy at elevated temperature in the range below the melting point of said solvent metal and above the minimum temperature for effective oxidation of said oxidizable metal to an oxygen containing environment to oxidation harden said alloy, decreasing the cross-sectional area of the oxidation hardened metal by cold working at least 75%, and forming a spring therefrom.

3. The process of making a spring of polycrystalline metal alloy hardenable by internal oxidation, said alloy having a solvent metal selected from the group consisting of silver, copper, palladium and nickel and an oxidizable metal dissolved therein in an amount ranging between 0.05% and 0.35%, comprising the steps of subjecting said alloy at elevated temperature in the range below the melting point of said solvent metal and above the minimum temperature for effective oxidation of said oxidizable metal to an oxygen containing environment to oxidation harden said alloy, decreasing the cross-sectional area of the oxidation hardened metal by cold working at least 75%, annealing said alloy, and forming a spring therefrom.

15

References Cited in the file of this patent

UNITED STATES PATENTS

|           |             |                |
|-----------|-------------|----------------|
| 2,015,509 | Austin      | Sept. 24, 1935 |
| 2,493,951 | Mari et al. | Jan. 10, 1950  |
| 2,539,298 | Doty et al. | Jan. 23, 1951  |
| 2,932,595 | Pfluum      | Apr. 12, 1960  |

FOREIGN PATENTS

|         |        |               |
|---------|--------|---------------|
| 542,630 | Canada | June 23, 1951 |
| 533,137 | Canada | Nov. 13, 1956 |

OTHER REFERENCES

Transaction AIME, vol. 147, pp. 205-221, 1942.